

## UNITED STATES PATENT OFFICE

2,267,565

## DYESTUFFS

Talfryn James and David Charles Forsht, Lock Haven, Pa., assignors to American Aniline Products, Inc., New York, N. Y., a corporation of New York

No Drawing. Application June 27, 1938,  
Serial No. 216,066

1 Claim. (Cl. 8—48)

This invention relates to the manufacture of dyestuffs and their application to artificial silks, and it is particularly concerned with dyeing cellulose acetate silks with dyestuffs which yield a color ranging from a jet black to a green blue. The invention provides a novel dyestuff for such silks which is of peculiar advantage in carrying out dyeing operations.

In dyeing cellulose acetate material with dyes of this type, it is difficult rapidly to distribute and secure the full color throughout the fibres of the yarn, by reason of the slow manner in which the fibres absorb such dyes. This is particularly true of heavy fabrics, the fibres of which are reached and penetrated with extreme difficulty.

The slowness with which dyeing operations of this type are at present carried out is a considerable handicap to commercial practice. Present day requirements call for speed in dyeing in order to meet demands for immediate deliveries caused by rapid style changes.

Moreover, relatively high concentrations of color must be maintained in the dye bath in order

5 As a specific example of one way in which we may prepare a dyestuff, we dissolve 1 mol of para nitroaniline in an excess of concentrated hydrochloric or sulphuric acid and cool the solution to a temperature below 25° C. We then stir in a solution of sodium nitrite sufficient to diazotize completely the para nitroaniline. This diazotized compound is intermixed with an aqueous solution of phenyl diethanolamine at any temperature within the approximate range of —10 to +40° C., either in a neutral or alkaline state, by the addition of an alkaline compound such as caustic soda, sodium acetate, sodium phosphate, or sodium carbonate. The dyestuff thus formed may be filtered and reduced with a concentrated solution of a sulphide such as sodium sulphide, or the reduction may be carried out in the coupled suspension without filtration. The final dyestuff is then filtered, washed, dried and pulverized.

10 The manner in which the reaction proceeds will be observed from the following structural progression:



15 to drive the dye into the fibre. After the dyeing is complete, considerable quantities of unabsorbed dyestuffs are left in the bath, which is wholly wasted unless the dyer has additional orders for that particular colored yarn, in which case he can use the partially spent bath only by fortifying it with additional dyestuff.

20 Objects of the invention are to overcome these difficulties and to provide a color which will be rapidly absorbed by the material to be dyed and which will be almost completely absorbed therein, and thus to speed up production materially and at the same time effect large economies by avoiding waste of dye bath ends.

In general, the invention consists in diazotizing aromatic nitro amines and their substituted derivatives, such as chlor, or brom, etc., and coupling the diazo compound thus prepared with mono hydroxy ethyl, di hydroxy ethyl, mono hydroxy ethyl ethyl derivatives of aromatic amines or their substituted derivatives. The compound to be coupled with the said diazo compound generally contains an aliphatic radical such as methyl, ethyl or a higher straight chain compound.

25 This product dyes cellulose acetate filaments with great rapidity and permits increased production in machine or jig dyeing treatments. Furthermore, the acetate fibres take up the dye so well that the dye bath is exhausted practically completely, thereby eliminating waste in the spent dye bath.

30 The novel dyestuff is also of advantage in the dyeing process which generally proceeds by adding the required weight of dyestuff to a solution of soap, alkali, and a dispersing agent such as Turkey red oil. This suspension is brought to the boil, cooled with cold water to a temperature generally below 70° C. The material to be dyed is entered into the bath after it has been wetted out. The temperature of the dye bath is raised to about 75—80° C. and the dyeing permitted to proceed until the required depth of color is obtained, or the dye bath exhausted. The material is then withdrawn, well washed with water and immersed in a bath containing sodium nitrite, to which is then added an acid, in general practice either hydrochloric acid or sulphuric acid, at ordinary temperature.

The material is allowed to remain in this bath for about twenty minutes, after which it is taken out, well washed and the color developed by immersing the material at a temperature of about 35° C. in a bath made up of beta hydroxy naphthoic acid, or its derivatives, dissolved in the required amount of alkali such as caustic soda, and acidified with an acid such as formic acid to such an extent as to retain the naphthoic acid derivative in solution.

The temperature is then raised to about 60° C. and the bath held at this temperature for roughly thirty minutes. The material is then taken out, well washed, soaped, well washed again, and dried.

We have found that in the development of the color as above outlined by beta hydroxy naphthoic acid or its derivatives, the particular dyestuff of the present invention reacts peculiarly to give varying shades of color, varying from a green blue to a jet black, depending solely on the amount of dyestuff available for the developing reaction. This is not true with ordinary black dyes, for although there may be more than one compound formed during the developing reaction, only one shade of color is produced thereby. Accordingly, in addition to the advantages of rapid and efficient dyeing, we obtain the advantage that we can greatly increase the range of color obtainable by this single dyestuff simply

by varying the amount thereof available for reaction with the beta hydroxy naphthoic acid solution.

As an example of the way in which these different results are accomplished, we take four percent. of para amino benzol azo-dihydroxyethyl-aniline, calculated on the weight of the material to be treated, and follow out the dyeing procedure outlined above until the developing step is 10 reached. We then treat the dye-impregnated material with a weight of beta hydroxy naphthoic acid calculated as one percent. of the weight of the material treated. The color develops into a green blue. If, however, we use 10% of black 15 dye and 1% of beta hydroxy naphthoic acid, we obtain a jet black.

Having thus described our invention, what we claim is:

The process of treating cellulose acetate which 20 comprises applying to said material para-amino benzol-azo-dihydroxyethyl-aniline in an amount of from 4% to 10% by weight of the acetate, then diazotizing the dyestuff upon the material and coupling thereon from a solution beta-hydroxynaphthoic acid, the amount of the coupling 25 component being 1% by weight of the acetate so as to produce thereon a shade ranging from green blue to blue and jet black.

TALFRYN JAMES.

DAVID CHARLES FORSHET.